

## UNITED STATES PATENT OFFICE

2,242,960

## PRODUCTION OF MOTOR FUEL

Alexander N. Sachanen and Arlie A. O'Kelly,  
Woodbury, N. J., assignors to Socony-Vacuum  
Oil Company, Incorporated, New York, N. Y., a  
corporation of New York

No Drawing. Application August 27, 1938,  
Serial No. 227,106

4 Claims. (Cl. 260—671)

This invention relates to the production of alkyl aromatic compounds by reacting aromatic and olefinic hydrocarbons. More particularly, the invention relates to a process for the production of alkyl aromatic hydrocarbons of high anti-knock value which are of suitable boiling range for use as motor fuels.

Processes for the cracking of gas oil and similar petroleum fractions to gasoline result in the production of hydrocarbons boiling within the gasoline range, and also result in the production of a considerable amount of lighter, normally gaseous hydrocarbon products. Appreciable quantities of these lighter gaseous products are olefinic and unsaturated in nature. Appreciable quantities of the gasoline-like condensate are also olefinic in nature. Processes of this nature result in the production of gasolines of varying qualities with respect to anti-knock characteristics, dependent upon both the charging stock originally processed and upon the nature of the process of cracking through which it has been passed.

Many of the liquid gasoline-like products of such cracking processes are relatively high in anti-knock characteristics when judged from the standpoint of the requirements of an automobile motor. Few of them, however, even approach the possession of sufficiently high anti-knock characteristics to permit of their use, as produced, in more advanced high compression type of engines, as for example the engines designed for use in aviation.

Alkylated benzenes boiling within the boiling range of commercial gasoline are known to be capable, when mixed with gasoline, of imparting to the mixture a high degree of anti-knock capability. Various methods for the production of alkylated benzenes by combining olefinic or similar unsaturated material, either from the products of a conventional cracking process or from other sources, with aromatic compounds of the nature of benzene or its homologues have been proposed.

The proposed prior processes, in general, take the nature of catalytic condensation reactions carried out at comparatively low temperatures in the presence of condensation catalysts. For example, such catalysts as aluminum chloride, various other metallic chlorides, sulfuric acid, phosphoric acid, and the like, are used at low temperatures, i. e. temperatures of the nature of 30° to 350° F. (about -1° C. to +177° C.). It has also been proposed to pass cracked gasoline in company with the normally gaseous materials

produced during cracking, together with benzene, through condensing catalysts of the nature of fuller's earth, at these low temperatures. However, at such low temperatures clay-like catalysts do not appear to exert much, if any, catalytic action, and, as the reaction does not proceed appreciably at these low temperatures without the use of a catalyst, other catalysts, such as sulfuric acid, etc. are generally used.

In general, the catalytic processes conducted at low temperatures are open to many objections. One of the principal disadvantages of such processes when employing the usual low-temperature reactive catalysts, such as metal chlorides, sulfuric acid and phosphoric acid, is that the consumption of catalytic material is relatively high, and, if not entirely consumed, a complicated and costly process of regeneration is required. Many of these catalytic materials are corrosive to the materials of construction normally used, and introduce this, as well as other operating difficulties.

A more serious objection, however, to processes carried out at low temperatures for the alkylation of aromatic compounds to form compounds to be added to gasoline, is that of low yield of products distilling in the boiling range of gasolines. The low yield is caused, in the main, by a considerable amount of the raw materials forming compounds of higher boiling range which are not usable in gasoline, and are particularly unsuitable for use in gasolines of the lower boiling-point type, such as gasolines of aviation grade and the like. Since any condensation catalyst will not only bring about the joining of a single alkyl radical with an aromatic radical, but will also, more or less, effect polymerization reactions among the alkyl radicals themselves, as well as the condensation of several alkyl radicals with a single aromatic radical, it may be seen that the possibilities of loss of yield from this source may be quite high.

It is an object of this invention to provide a highly efficient process for the production of alkyl aromatic compounds.

Another object of this invention is to provide a highly efficient process for the production of alkylated aromatic compounds which possess a high anti-knock value and are of suitable boiling range to be used in motor fuels.

A further object of this invention is to provide a highly efficient process for the production of alkylated aromatic compounds which affords optimum conditions for the formation of alkylated aromatic compounds of a desired boiling range

and minimizes the formation of alkylated benzenes without the desired boiling range and, furthermore, acts to reduce compounds of undesired boiling range, if formed, to compounds of the desired boiling range.

Still another object of this invention is to provide a process for the production of alkylated aromatic compounds wherein such catalysts as various clays and the like may be used with a high degree of success.

This invention is based upon the discovery that the reactions between unsaturated or olefinic materials and aromatic materials to produce compounds of the alkyl benzene type which are within the gasoline boiling range are remarkably improved and, moreover, give commercially feasible yields even in cases where no perceivable reaction occurs under more moderate conditions of operation, when the reactions are carried out at high temperatures of the nature herein disclosed and under suitable conditions tending to promote the condensation reaction. For instance, we have discovered that when the reaction is carried out at temperatures upwards of about 400° C., catalytic materials promote the reaction to an unusual degree and under optimum conditions as when elevated pressures are also used, practically a theoretical yield of aralkyl compounds within the gasoline boiling range may be obtained.

It is believed that the remarkably improved results derived from our invention are attributable to the fact that at the elevated temperatures of our process combined with the action of a suitable catalyst, not only will olefinic or similar compounds combine with aromatic materials to form alkylated aromatic compounds within the gasoline boiling range to an optimum degree, but that also under these conditions the formation of polymers of olefinic materials and of polyalkyl benzenes not within the gasoline boiling range is minimized and that such compounds, if formed, are immediately broken down into lower boiling compounds of an alkylated benzene nature which are within the gasoline boiling range.

The aromatic compounds with which our invention is concerned are of the nature of benzene, its homologues or compounds containing benzene nuclei. The aromatic compound (or mixture of aromatic compounds) may be employed in a relatively pure condition or they may be supplied by the use of products which are known to contain a substantial portion of these aromatic ingredients. Likewise the olefinic materials may be supplied as a relatively pure product or may be derived from the use of a product containing a substantial amount thereof. For instance, the olefinic material may be propylene, butylene, amylene, mixtures thereof, normally gaseous products of cracking, cracked gasolines or fractions of cracked gasolines containing olefines.

The catalyst employed should be highly selective in that it promotes alkylation reactions but is either a non-catalyst or a negative catalyst for other reactions. Catalysts usually do not act with perfect selectivity, hence normally one must choose a catalyst which acts predominantly in the desired manner. The catalysts which we prefer to use are of the clay type. In addition to the various clays themselves and the various activated clays, there are numerous other porous, refractory, adsorptive materials of similar nature which may be used and come under the common designation of clay type catalyst, for example,

fuller's earth, pumice and granular diatomaceous earth. Furthermore, it is to be understood that these various clay-type catalysts which have other catalytic materials impregnated therein or thereon or otherwise conjoined for use may be employed. In general, any alkylation catalyst which is active at the temperature of our reaction may be used. However, it is to be noted that the normally used catalysts of low temperature processes, such as aluminum chloride, sulfuric acid, etc. cannot be used in our high temperature process.

Since the alkylation reaction, together with the attendant cracking reactions which are present at the temperatures herein disclosed, bring about a gradual poisoning or deterioration of the catalyst by the deposit of carbon and carbonaceous impurities thereon, it is well to use a clay which is possessed of a sufficiently refractory nature so that it may be regenerated in situ by burning; in fact, some of the clay catalysts used by us have been regenerated as many as 8000 times and are still quite satisfactory. Because of the ease with which the clay-type catalysts may be regenerated, they afford a substantial advantage in their use. It is also well to use clay particles of such physical nature with respect to size and dimension that they may be effectively packed together in a catalytic mass and yet, at the same time, present a sufficient cross-sectional area of flow that the reactants may have a ready passage therethrough as well as a suitable exposure of catalytic material to reactants. A convenient and efficient form for the catalyst is small granules, rods or cylinders.

The use of clay-type catalysts has many distinct advantages in addition to those already named. For instance, the clay is not corrosive to the normal apparatus as are the usual alkylation catalysts and, furthermore, there is a relatively small consumption of the clay catalyst during operation as contrasted to the relatively high consumption of catalyst which is usually encountered. It is to be noted that our process alone appears to afford suitable conditions for the satisfactory use of clay catalyst since under more moderate conditions of operation the clay appears to be relatively ineffective as a catalyst.

The temperatures employed in our process should be sufficiently high to be capable of producing at least a partial cracking of the hydrocarbons having boiling points higher than the gasoline boiling range, as, for instance, temperatures upwards of about 400° C., and it is desirable to maintain the temperature between about 400° C. and 600° C., since above 600° C. the results are less satisfactory. In the preferred process the temperature is maintained between 400° C. and 500° C. as the most favorable results are obtained in this range with temperatures of 450 to 500° C. being optimum.

In our catalytic process any increase in pressure above atmospheric appears to enhance the reaction until at about 100 atmospheres, using a clay catalyst, practically optimum conditions are reached as the yield then closely approaches the theoretical. Hence, in practice, it is preferred to maintain the pressure within the range of pressures between about 50 and about 100 atmospheres. It is to be understood, however, that pressures above 100 atmospheres and up to about 250 atmospheres may likewise be used with good results. Above 250 atmospheres the results become less favorable as there is an increase in

the production of heavy molecules above the gasoline boiling range.

The differences found between the reactions carried out in accordance with our process and those which may be carried out at the temperatures heretofore thought to be appropriate may be shown by the following experiments wherein the mixtures of amylene and toluene were treated at a reaction temperature of 890° F. (about 470° C.) for a time of fifteen minutes.

At atmospheric pressure and in the absence of a catalyst, no reaction products of the nature of alkylated benzenes were detectable in the effluent.

At atmospheric pressure in the presence of a highly activated porous adsorptive catalyst of the clay type, reaction products indicated that 45% of the theoretical yield of alkylated benzene products could be obtained.

At a pressure of 1500 pounds per square inch with the catalyst, a reaction yield of 58% of the theoretical was obtained.

At a lower temperature range of 400 to 600° F. (about 205 to 315° C. which is much higher than the customary alkylating temperature) even in the presence of a highly active catalyst of the clay type, no measurable rate of reaction was found.

To further point out the differences between the prior art and the present invention, we may discuss the reactions involved. For example, when benzol is condensed with amylene, the following reaction takes place:



and with butylene:



These are the simplest reactions possible under these circumstances, and, as may be observed, result in each case in the alteration of benzol, which has a boiling point of 194° F. (within the aviation gasoline boiling range) to an amyl benzene, which has a boiling point of 401° F., and to butyl benzene, which has a boiling point of 356° F., respectively, both of which are barely within the upper limits acceptable for ordinary motor fuel, and which are unacceptable for use in lighter gasolines, as, for example, aviation gasoline wherein the demand for anti-knock capability is particularly great. Note that the above takes no account of the known formation of a considerable proportion of the olefines into polymerized products of doubtful anti-knock value, and of the known formation of poly-alkylated aromatics of considerably higher boiling ranges not capable of being used in any type of gasoline.

In contrast, the reaction of benzene with amylene and butylene at the high temperatures of our process herein described are mainly of the following nature:

I—With amylene:



II—With butylene:



These two compounds formed, namely propyl- and ethyl-benzene, boil respectively at 310° F. and 284° F. and both may be used even in the low-boiling types of gasoline, such as aviation gasoline. These differences in the type of reaction encountered are especially striking when the material from which the alkylating compounds

are derived is gasoline or a mixture of gasoline and cracking vapors, because many of the olefines present, particularly those derived from the gasoline, are high molecular weight olefines, and many of them are olefines of a complicated nature quite prone to polymerization, as is evidenced by their capability of gum formation, and the like, and by their ability to polymerize to materials of boiling point higher than gasoline under the relatively simple treatment encountered in the vapor phase degumming processes in contact with fuller's earth.

With increases in temperature this difference in the type of reaction becomes more striking, since with increases in temperature there is a rapidly increasing tendency to break up the aliphatic radical, resulting in the production of alkylated benzenes containing very short and simple alkyl radicals, such as toluene, ethyl benzenes and propyl benzene and, consequently, resulting not only in the production of a greater amount of alkylated benzenes within the boiling range of aviation gasoline, but also in a much more efficient utilization of the aromatic radicals present.

The process may be carried out either as a batch operation or the process may be made continuous by employing a pipe still and a reaction chamber.

The effectiveness of this method of operation, and the effect of the several variables, may be seen from a consideration of the following examples, in each of which one or more of the operating principles herein disclosed is applied. It is to be understood that these examples are merely for purposes of illustration and not to be construed as limiting the invention in any sense.

#### Example I

Toluene is alkylated with amylene in the presence of a porous adsorptive catalyst comprising activated clay at a temperature of 840° F. (about 449° C.) and under a pressure of 1250 pounds per square inch gauge (about 83.3 atmos.) for a period of 45 minutes (batch operation), the total yield of alkylated aromatic hydrocarbons is 100% of that which might theoretically be expected, and of these alkylated aromatic hydrocarbons 69% are within the gasoline boiling range.

#### Example II

Toluene is alkylated with amylene by passing the mixture over a similar activated clay catalyst at a temperature of 885° F. (about 474° C.) and at a pressure which is substantially atmospheric (batch operation). The total yield of alkylated toluenes is 57% of that which might theoretically be expected, and of these alkylated toluenes 70% are within the gasoline boiling range.

#### Example III

Benzene is alkylated with butylene in the presence of a similar activated clay catalyst at a temperature of 850° F. (about 454° C.) at a pressure of 1500 pounds per square inch gauge (100 atmos.) for a period of fifteen minutes (batch operation). The total yield of alkylated benzenes is 74% of that which might be expected, and of these alkylated benzenes over 80% are within the gasoline boiling range.

#### Example IV

Benzene is alkylated continuously (in a pipe still with a reaction chamber) with cracked gases from stabilization containing 21% propyl-

ene and 17% butlenes in the presence of a clay catalyst. The above mixture of liquefied gases and an excess of benzene is charged to the pipe still at 975° F. under a pressure of 1500 lbs. per square inch gauge in a once-through process. The total yield of alkylated benzenes is 96% of that which might be expected, and of these alkylated benzenes 86% are within the boiling range of motor gasoline, s. g. 0.870.

We claim:

1. A process of preparing alkyl aromatic compounds in the gasoline boiling range which comprises alkylating aromatic hydrocarbons with olefine hydrocarbons at a temperature between about 400° C. and about 600° C. in the presence of a catalyst comprising an association of silicon oxide and aluminum oxide and under a super-atmospheric pressure. 15

2. A process of preparing alkyl aromatic compounds in the gasoline boiling range which com- 20

prises alkylating aromatics with olefines at a temperature between about 400° C. and about 600° C. in the presence of a clay catalyst.

3. A process of preparing alkyl aromatic com- 5 pounds in the gasoline boiling range which comprises alkylating aromatics with olefines at a temperature between about 400° C. and about 600° C. in the presence of a clay catalyst and under a pressure between about 50 and about 10 250 atmospheres.

4. A process of preparing alkyl aromatic com- 15 pounds in the gasoline boiling range which comprises alkylating aromatics with olefines at a temperature between about 400° C. and about 500° C. in the presence of a clay catalyst and under a pressure between about 50 and about 100 atmospheres.

ALEXANDER N. SACHANEN.  
ARLIE A. O'KELLY.